

## UNITED STATES PATENT OFFICE

2,545,138

## CORROSION INHIBITING COMPOSITIONS

Werner David, Chester, England, assignor to Shell Development Company, San Francisco, Calif., a corporation of Delaware

No Drawing. Application February 2, 1948, Serial No. 5,907. In Great Britain June 30, 1947

9 Claims. (Cl. 252—33)

1

This invention relates to compositions having ability of displacing moisture, corrosive materials and the like from corrosive surfaces. This invention also pertains to the formation on such surfaces of a non-corrosive moisture resistant protective film. More particularly this invention pertains to corrosion inhibiting compositions suitable for protecting metal and non-metal surfaces by rendering them impervious to water, electrolytic solutions, corrosive fluids, gases, and the like, by displacing said contaminant from said surfaces and forming thereon a tenacious protective film having good lubricating properties.

It is well known that moisture, corrosive fluids and gases, e. g.  $H_2S$ ,  $SO_2$ , etc., readily attack not only metallic surfaces but non-metallic surfaces and cause corrosion, rusting, pitting and other damage to such surface. Also, aqueous solutions when in contact with a metallic surface readily attack it and cause corrosion and rusting. Under certain conditions the problem of corrosion becomes exceedingly serious because once started it is progressively accelerated. Thus, oils containing small amounts of water become very corrosive to metals in contact therewith. This is due to the fact that oils and particularly liquid petroleum hydrocarbons are very good solubilizers of oxygen, and any moisture present therein becomes surrounded by an almost inexhaustible source of oxygen. Moisture under such conditions is inhibited from evaporating and, since the rate of transfer of oxygen from hydrocarbons, such as mineral oil or gasoline, to water is limited, ideal conditions for rusting and corrosion are set up. The presence of electrolytes and formation of corrosive decomposition products in oils and the like also greatly increase the rate of corrosivity.

Under conditions where, in addition to those enumerated, elevated temperatures are encountered, corrosive activity is greatly accelerated. Thus moisture, salt sprays and other contaminants or acidic decomposition products and corrosive gases formed during operation of engines, such as internal combustion engines, Diesel engines, aircraft engines, turbines and various other machinery and industrial equipment, readily attack and rust or corrode contacting metal surfaces. The damage thus caused is not to the metal surface alone for rust particles frequently break off and enter the circulating system of engines and cause plugging, clogging, and fouling of conduit lines, columns, plates, and the like of cracking equipment, tubes, evaporators, etc.

Corrosion of alloyed bearings and other alloyed

2

surfaces due to contact with water can attain such an aggravated stage as to cause great fatigue stresses to be set up, which ultimately result in cracking of the metal.

5 The problem is equally serious when combating rusting and corrosion of steel drums, storage tanks used to store gasoline, hydrocarbon oils and the like. Moisture adhering to pickled steel, quenched steel, equipment such as instruments, engine starters and generators on landing crafts, hydraulic systems, machinery for metal processing and the like are also extremely susceptible to corrosion and must be protected.

Rust preventative, water displacing compositions are particularly desired in metal rolling operation such as prior to cold rolling of metals. Generally, prior to cold rolling, metal sheets or strips are hot rolled, and then subjected to the following operations:

15 20 (a) A pickling operation wherein, if desired, an inhibitor is added to the pickling bath;  
(b) A washing of the steel sheet or strip to remove the pickling agent;  
(c) A drying of the sheet or strip, for example,

25 by means of a hot air blast; followed, if desired by

(d) An oiling treatment to inhibit corrosion, particularly if the metal thus treated is to be stored for some time prior to cold rolling.

After the material has been subjected to these operations it is cold rolled, generally using, as a lubricant and cooling agent, a soluble oil emulsion. Subsequently, the articles are annealed, and then subjected, if desired, to a light rolling without oil through highly polished rolls. The object of this step is to confer some degree of hardness to the metal and also to burnish it, thus producing a pleasing polished appearance.

The cold rolling process carried out in the above described manner suffers from various drawbacks. Washing, drying and oiling operations are expensive in time, labor, and cost, and moreover, unless the oil composition is carefully selected it is frequently found to be the cause of staining after the article has been annealed and this is probably caused by catalytic decomposition of oil vapors on the metal surface being annealed.

From the above description of metal rolling it can readily be appreciated that simplification of the process by elimination of the drying, washing and subsequent oiling step is greatly desired. This can be accomplished by use of water-displacing compositions of this invention prior to the cold rolling step.

In order for water displacing compositions to be effective they must act rapidly and thereafter spread uniformly and quickly over the surface treated, adhere tenaciously thereto and protect the surface from corrosion. In addition, water-displacing compositions should possess the following properties:

- (1) They should be immiscible with water;
- (2) They should be stable under all conditions of use or in storage;
- (3) They should be non-reactive with contacting surfaces being treated;
- (4) They should provide protection to the surface treated for long periods of time;
- (5) They should possess some degree of lubricity; and
- (6) They should not cause staining or marring of the surface.

Countless materials and compositions have been tried for protecting surfaces, such as metal surfaces, against damage caused by water, corrosive fluids and the like by forming on said surface a non-reactive corrosion protective film having lubricating properties. Metal surfaces have been coated or treated with greases, fatty compositions, waxes, organic compounds, e. g. organic acids, amines; inorganic compounds and the like in order to protect them against corrosion. In almost all cases where no chemical reaction occurred between the surface treated and the corrosion or rust inhibitor very little benefit is derived. This is due to the fact that non-chemical reactive inhibitors are incapable of penetrating the surface being protected and are incapable of displacing the contaminant therefrom. In cases where such inhibitors are able to form protective coatings on surfaces they are easily displaced by moisture or rupture readily. They are relatively ineffective against corrosive acidic materials and hot gases such as are formed during operation of combustion and turbine engines and are easily destroyed when applied to surfaces which are subjected to high temperatures.

It is an object of this invention to protect metal surfaces in contact with corrosive contaminants against corrosion by treating said surfaces with a composition having the property of displacing said contaminants from said surface and forming thereon an impermeable tenacious protective film. It is another object of this invention to protect metallic surfaces with a water displacing, water resistant non-corrosive protective film having no detrimental effect upon the metal surface treated. It is still another object of this invention to provide metal surfaces with a water and acid resistant film which is not susceptible to rupture even at elevated temperatures and which could be readily removed when desired. Still another object of this invention is to form protective film on metal surfaces which are not detrimental to contacting fluids and which do not interfere with their function as lubricants, hydraulic fluids, quenching agents and the like. Another object of this invention is to form a composition of matter capable of protecting metal surfaces from corrosion, said composition also possessing lubricating properties. Another object is to form film-forming metal protective compositions which are stable and readily miscible with petroleum hydrocarbons such as lubricating oils or other inert organic carriers and the like. It is also another object of this invention to treat surfaces whether metallic or non-metallic so as to form thereon a protective film which is impervious to moisture

15

20

25

30

35

40

45

50

55

60

65

70

75

and corrosive fluids, and which can be readily removed when desired. Other objects will be apparent from the following description.

It has now been discovered that various metals and other materials subjected to corrosive influences can be protected simply and effectively by treatment with a composition of matter comprising essentially a blend comprising a major amount of a hydrocarbon and/or mixtures of said hydrocarbons, synthetic lubricants, fixed fatty oils and the like, and minor amounts of specially selected wetting agents, spreading agents and film-forming agents. The additives of this composition must be present in a rather critical amount, and must be present at all times during the active life of the composition in order to function as an effective water displacing, non-corrosive, protective film-forming composition.

The dispersing medium is substantially a water-immiscible hydrocarbon or a mixture of hydrocarbons such as petroleum oils or other type of oils, or their derivatives. These carriers or dispersing mediums are preferably derived from petroleum hydrocarbons and may include various petroleum naphtha cuts, mineral spirits, lubricating oil distillates, mineral seal oil, kerosene, gas oils, mineral lubricating oil, transformer oil, white oil, kerosene SO<sub>2</sub> extract, aromatic solvents, petroleum ether, aromatic hydrocarbons such as benzene, p-xylene, o-xylene, m-xylene, cumene, butyl benzene; paraffinic hydrocarbons, e. g. normal hexane, dimethyl pentane, octane, nonane, undecane, dodecane; cycloparaffin, e. g. cyclohexane, methylcyclohexane, isopropylcyclohexane; synthetic oils such as polymerized alkylene oxides, polymerized olefins, esters, e. g. 2-ethylhexyl sebacate, etc. The dispersing medium is usually present in amounts of between about 85% and about 95% of the composition, depending upon its viscosity, penetrability and particular application or condition under which it is used. Preferably, the base oil should not exceed a viscosity of about 65 seconds Redwood I at 140° F., and should contain little or no free or combined sulfur.

Additives which have the power of wetting metal and like surfaces and of displacing moisture and other contaminants therefrom so as to allow direct contact and adherence of the protective agent to the surface, are salts of sulfonic acid such as ammonium, amine, alkali, alkaline earth and heavy metal salts of petroleum sulfonic acid derived from substantially light petroleum fractions rich in aromatics, preferably having an aromatic content between 5% to 10%. Particularly suitable for forming the sulfonates are petroleum naphthas, kerosene, transformer oils and the like. The sulfonates can be formed by any conventional means. For example, petroleum naphthas or kerosene fractions rich in aromatics can be treated with suitable amounts of sulfuric acid to obtain sulfonic acids. These acids can be recovered by alcoholic extraction and thereafter neutralized with alkali to form the alkali metal salts of these sulfonic acids. Sulfonates produced from lubricating oil fractions as well as other petroleum hydrocarbons are generally inferior to the above preferred hydrocarbons as sources for the sulfonates to be used in combination with the other additives of this invention. Also, sulfonates derived from alkylated aromatic e. g. butyl naphthalene sulfonate, diwax benzene sulfonate, and the like, can be used. If desired various other salts of said sulfonic acids can be used.

Instead of using the sulfonates derived from light petroleum fractions as the sole wetting agent, other well known wetting agents can be used in combination therewith. Among them can be included esters and various salts of organic compounds containing a minimum of 8 carbon atoms in the molecule. Particular examples are soap or salts of fatty materials or petroleum acids obtained by oxidizing paraffin waxes, the alkali and alkaline earth metal salts, e. g. sodium, potassium, calcium or magnesium salts of wool grease, degras fatty acid, oleic acid, stearic acid, petroleum acids; alkali salts of sulfated alcohols having between about 8 to 20 carbon atoms in the molecule, e. g. sodium oleyl sulfate, sodium lauryl sulfate, sodium oceanol sulfate, ammonium lauryl sulfate; neutralized alkylated aromatic

5

10

15

thereof are cottonseed oil, rape oil, menhaden oil, sardine oil and the esters thereof.

Any of the above oils can be blown by conventional means such as by air at elevated temperatures until the oil has attained the desired consistency. Usually blowing is stopped when the product has obtained the consistency of castor oil. Blowing has a profound effect upon the treated oil. Thus by the action of oxygen or air, a part of the unsaturated acids present in said oils is changed to naphtha-insoluble oxy-acids; another part decomposes into volatile acids of low molecular weight which are eliminated; and a considerable amount of polymerization, as well as lactone formation occurs. The changes which occur by blowing oils can best be illustrated by reference to Table I.

Table I

|                      | Sp. Gr. at<br>15° C. | Iodine<br>Value | Sap. Value | Per cent<br>oxy-acids<br>insoluble in<br>petroleum<br>ether |
|----------------------|----------------------|-----------------|------------|-------------------------------------------------------------|
| Pure rape oils       | 0.913 to 0.917       | 94 to 106       | 170 to 179 | 0                                                           |
| Blown rape oils      | 0.968 to 0.975       | 47 to 52        | 209 to 217 | 24 to 27                                                    |
| Pure cottonseed oil  | 0.922 to 0.925       | 108 to 110      | 191 to 198 | 0                                                           |
| Blown cottonseed oil | 0.972 to 0.979       | 56 to 65        | 214 to 225 | 26 to 29                                                    |

sulfates; and alkali salts of mono- and poly-alkyl esters of sulfodicarboxylic acid, e. g. sodium salt of diamyl sulfo succinic acid, sodium salt of dilauryl sulfo succinic acid, disodium monocetyl monosulfo succinate, etc.

The wetting agents of this invention, such as alkali sulfonates derived from low boiling petroleum hydrocarbons rich in aromatics when used alone or in combination with other wetting agents referred to above, possess the unique property of displacing moisture from metal surfaces and in addition act as powerful penetrants, which however are readily displaceable by the protective film-forming agent of this invention. This is apparently due to the fact that these wetting agents are substantially miscible with and have a great affinity for water, enabling them to remove moisture from the metal surface and allowing the penetrant and protective film-forming agent to come in direct contact with the surface being treated.

The amount of preferred sulfonate wetting agent, which may be ammonium or sodium sulfonate, referred to above, when used either alone or in combination with other wetting agents varies between about 2% and about 5%, and preferably between about 2% and about 3%, by weight. When in combination with other wetting agents it is generally preferred to employ predominant amounts of the petroleum sulfonate.

The protective film-forming, water-displacing agents of this invention are blown or thickened animal, vegetable and/or fish oils and derivatives thereof, such as the full or partial esters of said oil. Among such esters may be included the mono, di and/or triglycerol ester of capric, lauric, myristic, palmitic, stearic, arachidic, behenic, oleic, linolein, ricinoleic acids and the like. These esters may be simple or mixed. In addition other fractions of said oils which are unsceptible towards a blowing treatment may be used. Oils which are suitable for use include: cottonseed oil, rape oil, kapok oil, corn oil, soya bean oil, pumpkin seed oil, beechnut oil, mustard oil, rice oil; seal oil, whale oil, menhaden oil, sardine oil, cod liver oil, neat's-foot oil, tallow oil, lard oil, and the like. The preferred oils and derivatives

30 displacing moisture from metallic surfaces and forming thereon a tenacious protective film. Just how blown oils perform this function is not exactly understood but it is believed that the polar groups formed during blowing have a strong affinity for water, allowing the rest of the material to adhere tenaciously to the metal surface and form a protective film thereon.

35 The protective film-forming water-displacing agents are generally used in amounts varying from 3% to 5% by weight.

40 To aid in spreading the film-forming metal protective agent evenly, minor amounts of cyclo-alkanols having between about 5 to 19 carbon atoms in the molecule and preferably between 45 about 4 to 8 carbon atoms, are added to compositions of this invention. Cyclic alcohols may include cyclohexanol, 4-tertiary amyl cyclohexanol, di-tertiary amylcyclohexanol, methylcyclohexanol, amylocyclohexanol, dimethylcyclohexanol, naphthenic alcohol, cyclobutanol, amyl cyclobutanol, quinitol, carvomenthol, menthol, beta and alpha terpineol, terpin and derivatives of cyclic alcohols such as obtained by intermolecular dehydration of an alkitol to produce polyhydric cyclic ethers. By an alkitol is meant a polyhydric alcohol having at least four carbon atoms and at least four hydroxy groups such as erythritols, pentitols, sorbitol, mannitol, and the like. The cyclic alcohols need not be used in amounts above 50 about 10% by weight and usually range from 5% to 10% although under certain conditions they need not exceed 5% by weight. The alcohols function as spreading agents. Thus once the wetting agent with the aid of the penetrant succeeds 55 in wetting the surface and removing the moisture or other contaminant, the alcohol helps spread uniformly the film-forming protective agent on to the treated surface.

60 All ingredients which constitute the present 65 composition must be present at all times. The absences of any one ingredient reduces the overall efficiency of the composition to such a degree as to render it almost useless as a moisture displacing corrosion inhibiting composition.

70 In order to more fully illustrate preferred com-

position of this invention, the following finished compositions are tabulated herein below and should not be construed as a limitation of this invention.

Table II

| Components               | Parts by Weight |    |     |    |    |    |
|--------------------------|-----------------|----|-----|----|----|----|
|                          | I               | II | III | IV | V  | VI |
| Mineral lubricating oil  | 91              | 90 | 89  | 86 | 90 | 89 |
| Sodium naphtha sulfonate | 2               | 3  | 2   | 5  | 2  | 3  |
| Blown rape oil           | 3               | 3  | 5   | 5  | 3  | 3  |
| Methyl cyclohexanol      | 4               | 4  | 4   | 4  | 4  | 4  |
| Oleic Acid               |                 |    |     |    | 1  | 1  |

The following table further illustrates compositions of this invention which are beneficial for displacing contaminants as described from various surfaces.

Table III

| Components <sup>1</sup>        |   |   |   |   |   |   |
|--------------------------------|---|---|---|---|---|---|
| Na petroleum sulfonate         | z |   |   |   | x | x |
| K petroleum sulfonate          |   | z |   |   |   | x |
| Ammonium petroleum sulfonate   |   | z | z |   |   | x |
| Na butyl naphthalene sulfonate |   |   |   | x |   | x |
| Na diwax benzene sulfonate     | z | z |   | x |   | x |
| Blown cottonseed oil           | z | z | z | x |   | x |
| Blown corn oil                 |   |   |   | x |   | x |
| Blown sesame oil               | z | z |   | x |   | x |
| Amyl cyclohexanol              |   |   |   | x |   | x |
| dimethyl cyclohexanol          |   |   |   | x |   | x |
| di-tert-amyl cyclohexanol      |   |   |   | x |   | x |
| cyclobutanol                   |   |   |   | x |   | x |

<sup>1</sup>The components listed can be dispersed in any suitable hydrocarbon such as mineral oil, kerosene, gas oil, mineral seal oil, mineral spirits and the like in an amount the total of which preferably does not exceed about 15% by weight.

The following example illustrates the applicability of compositions of this invention to the cold rolling of steel sheets or strips.

A hot rolled steel strip 5 $\frac{3}{8}$ " wide and 0.092% thick in coil form was passed continuously through a pickling bath which was maintained at between about 85°C. and 90°C. The pickled strip was then passed through a washing chamber where water was sprayed on said strip. It then is passed through a tank containing a composition of this invention preferable as noted in the Table II above, where all the water adhering to the strip is displaced. The displaced water settles rapidly out of the composition and is removed from the bottom of the tank at convenient times. The strips on leaving this tank pass through felt pads in order to remove excess oil adhering to the strip.

The strip is then cold rolled to 0.007" thickness. This rolling operation may be done immediately after the strip leaves the oil tank or the strip may be re-coiled and left to stand until rolling is convenient. After rolling, the strip is annealed in an electric furnace in an atmosphere of cracked ammonia gas at about 700°C.

The surface finish of strips treated as above are remarkably good and are greatly superior to the finish of similar steels treated by the usual process utilizing thermal dipping, oiling and soluble oil emulsion application during cold rolling. Furthermore surfaces treated with compositions of this invention are free from stains and other undesired deposits.

While the above example illustrates the preferred method of carrying out the process of cold rolling steel using compositions of this invention, various modifications can be made which may be apparent to those skilled in the art of steel rolling. Thus, such processes may be con-

tinuous or batch and the compositions of this invention may be applied by spraying, dipping, swabbing and the like.

Besides metal surfaces, materials such as rubber, electrical insulation materials, brake and clutch lining and the like may be treated with compositions of this invention whenever it is desired to displace water from them.

Although the essential ingredients which constitute compositions of this invention must be present, other additives can be included such as linear polymer thickeners, asphalts, pour point depressors, dyes, alkyl and alkylol amines, organic acid, e. g. oleic, stearic, cresylic naphthenic acids, phenolic compounds and the like. The addition of such additives are particularly desired when compositions of this invention are required to be used as temporary lubricants.

The present compositions may be applied to a surface to be protected by a means such as immersing, flooding, spraying, brushing, trowelling and the like. The protective film formed on said surfaces adheres tenaciously enough to withstand handling, light polishing, movement and high temperatures for long periods of time. It can be removed when desired by a suitable solvent or by simply rubbing with a cloth.

The present invention having thus been fully described is not to be limited by any specific examples which have been presented herein solely for the purpose of illustration, but only by the following claims.

This application is a continuation-in-part of my pending application Serial No. 734,875 filed March 14, 1947.

I claim as my invention:

1. A corrosion- and rust-inhibiting lubricating composition adapted to displace moisture from metal surfaces prior to being metal worked and prevent corrosion, said composition having the following formula and proportions:

|                                                                                                                   | Per cent by weight |
|-------------------------------------------------------------------------------------------------------------------|--------------------|
| Mineral lubricating oil                                                                                           | 85 to 95           |
| Sodium salt of petroleum naphthasulfonic acid derived from a petroleum naphtha containing from 5 to 10% aromatics | 2 to 5             |
| Blown rape oil                                                                                                    | 3 to 5             |
| Methyl cyclohexanol                                                                                               | 5 to 10            |

2. A corrosion- and rust-inhibiting lubricating composition adapted to displace moisture from metal surfaces prior to being metal worked and prevent corrosion, said composition having the following formula and proportions:

|                                                                                                                     | Per cent by weight        |
|---------------------------------------------------------------------------------------------------------------------|---------------------------|
| Mineral lubricating oil                                                                                             | From about 85 to about 95 |
| Ammonium salt of petroleum naphthasulfonic acid derived from a petroleum naphtha containing from 5 to 10% aromatics | From about 2 to about 5   |
| Blown rape oil                                                                                                      | From about 3 to about 5   |
| Methyl cyclohexanol                                                                                                 | From about 5 to about 10  |

3. A corrosion- and rust-inhibiting mineral lubricating oil composition adapted to displace moisture from metal surfaces containing a total not exceeding about 15% by weight, and each additive being in about equal proportions of sodium salt of petroleum naphtha sulfonic acid derived

from a petroleum naphtha containing from 5 to 10% aromatics, blown rape oil and methyl cyclohexanol.

4. A corrosion- and rust-inhibiting mineral lubricating oil composition adapted to displace moisture from metal surfaces containing a total not exceeding about 15% by weight and each additive being in about equal proportions, of ammonium salt of petroleum naphtha sulfonic acid derived from a petroleum naphtha containing from 5 to 10% aromatics, blown rape oil and methyl cyclohexanol.

5. A corrosion- and rust-inhibiting mineral lubricating oil composition adapted to displace moisture from metal surfaces containing a total not exceeding about 15% by weight and each additive being in about equal proportions, of salt of a petroleum sulfonic acid, blown vegetable oil and cycloalkanol.

6. A corrosion- and rust-inhibiting mineral lubricating oil composition adapted to displace moisture from metal surfaces containing a total not exceeding about 15% by weight and each additive being in about equal proportions, of salt of a petroleum sulfonic acid derived from a petroleum naphtha containing from 5 to 10% aromatics, blown vegetable oil and cycloalkanol.

7. A corrosion- and rust-inhibiting mineral lubricating oil composition adapted to displace moisture from metal surfaces containing a total not exceeding about 15% by weight and each additive being in about equal proportions, of salt of a petroleum sulfonic acid derived from a petroleum naphtha containing from 5 to 10% aromatics, blown fatty oil and cycloalkanol.

8. A corrosion- and rust-inhibiting light petroleum hydrocarbon lubricating composition adapted to displace moisture from metal surfaces prior to being metal worked containing a total not exceeding about 15% by weight and each additive being in about equal proportions, of salt of a petroleum sulfonic acid derived from a petroleum naphtha containing from 5 to 10% aromatics, blown fatty oil and cycloalkanol.

10 9. A corrosion- and rust-inhibiting liquid hydrocarbon lubricating composition adapted to displace moisture from metal surfaces prior to being metal worked containing a total not exceeding about 15% by weight and each additive being in about equal proportions, of a salt of a petroleum sulfonic acid derived from a petroleum fraction containing from 5 to 10% aromatics, blown fatty oil and cycloalkanol.

WERNER DAVID.

20

#### REFERENCES CITED

The following references are of record in the file of this patent:

25

#### UNITED STATES PATENTS

| Number     | Name         | Date          |
|------------|--------------|---------------|
| Re. 17,722 | Millring     | July 8, 1930  |
| 2,121,475  | Corkery      | June 21, 1938 |
| 2,182,992  | Lebo         | Dec. 12, 1939 |
| 2,348,715  | Adams et al. | May 16, 1944  |
| 2,359,738  | Schiermeier  | Oct. 10, 1944 |

#### FOREIGN PATENTS

| Number     | Country       | Date         |
|------------|---------------|--------------|
| 35 469,889 | Great Britain | Aug. 4, 1937 |